

Nov. 22, 1932.

A. SCHMIDT

1,888,891

PROCESS FOR MANUFACTURING BENT PIPES

Filed March 30, 1931



Fig. 1.



Fig. 2.



Fig. 3.



Fig. 4.



Fig. 5.



Fig. 6.

Inventor:  
A. Schmidt

By: Marks & Cleve  
A.H.Z.s.

## UNITED STATES PATENT OFFICE

ALFRED SCHMIDT, OF DUSSELDORF, GERMANY

## PROCESS FOR MANUFACTURING BENT PIPES

Application filed March 30, 1931; Serial No. 526,514, and in Germany May 31, 1930.

This invention relates to the bending of pipes such as are used for carrying media under pressure,—for example, steam, water and the like,—in such a manner that during the bending, outwardly projecting or inwardly directed folds are produced, and more particularly to the bending of such pipes to a curve of very small radius or the bending of pipes with very thick walls.

10 In my Patent 1,617,277, I have described a process for bending pipes in which individual parts at the inside of the bend to be produced were successively heated and the pipe was bent a small amount after each heating.

15 Other processes are possible for the manufacture of such pipe bends, for example, the bending of the pipe over a bending mold provided with depressions according to my patent application Serial No. 422,474 filed

20 January 21, 1930. Under ordinary circumstances these processes give very good results, but if the pipe to be bent has an unusually thick wall or if the bend to be produced has a very small radius of curvature, for ex-

25 ample, equal to the diameter of the pipe, the desired results as regards the shape of the folds, the shape of the pipe cross-section, and the elasticity of the pipe bend are very often not obtained.

30 These disadvantages are avoided by using in the manufacture of the pipe bend, partly one of the above-mentioned processes and partly a process such as is usual for bending smooth pipe bends, that is, a process in which the pipe is preferably heated over the whole circumference.

My new process consists in this that I first bend the pipe in the usual way to a smooth pipe bend of large radius of curvature and 40 then I proceed with the further bending according to one of the processes for making folded pipe bends, so that then the pipe acquires the desired radius of curvature. I may, however, carry out the operations in 45 the reverse order, that is, I may first use a process for producing folded pipe bends and afterwards one of the usual processes for producing smooth pipe bends. I may also use simultaneously the process which is usual 50 for producing folded pipe bends and that

which is usual for producing smooth pipe bends, the parts where the folds are to be formed being strongly heated and the other parts of the pipe walls being heated less strongly.

55 The heating of the folding places may be effected successively or also simultaneously for all the folds, or for individual groups of folds. Experiments have shown that by the use of my new process even with thick walled 60 pipes or with small radius of curvature a folded pipe bend is obtained which is quite satisfactory as regards shape of the folds and the cross-section of the pipe. The accompanying drawing illustrates examples of carrying out the process.

65 Figs. 1-3 show the process in which first a smooth pipe bend and then from it a folded pipe bend of small radius of curvature ( $r=D$ ) is produced.

70 Figs. 4-6 illustrate the manufacture of the same pipe bend, the folds first being produced on the pipe then the pipe being bent according to the usual process for making smooth pipe bends.

75 In Fig. 1 a pipe filled with sand is secured at 1. The part between the lines 2 and 3 is heated on all sides and then a tension is applied at 4, so that the pipe is bent in the shape shown in Fig. 2.

80 After cooling, the parts 5, 6, 7, 8, of the inner side of the curvature are heated successively and after each heating an outwardly projecting fold is produced by a tension at 4. The pipe bend shown in Fig. 3 is thus obtained.

85 Fig. 4 shows the same pipe filled with sand as Fig. 1. The parts 9, 10, 11, 12, are heated successively and after each heating a tension is applied at 4, the folds 13, 14, 15, 16, (Fig. 5) are then formed, while the heated parts bend. The part of the pipe between the lines 17 and 18 is then uniformly heated and brought into the shape shown in Fig. 6 by further tension at 4.

90 In the same manner pipe bends with inwardly projecting folds may also be produced.

95 What I claim is:

100 A process for bending pipes which are suit-

able to withstand internal pressure, comprising filling the pipe with sand and securing it, heating the whole circumference of the part to be bent and partly bending it allowing the pipe to cool, heating individual parts of the pipe walls on the inside of the bend, and bending the pipe a small amount after each heating until the desired shape is obtained.

18 In testimony whereof I have signed my name to this specification.

ALFRED SCHMIDT.

15

20

25

30

35

40

45

50

55

60

65